



US007981250B2

(12) **United States Patent**  
**Polverari et al.**

(10) **Patent No.:** **US 7,981,250 B2**  
(45) **Date of Patent:** **Jul. 19, 2011**

(54) **METHOD FOR PAPER PROCESSING**

(75) Inventors: **Marco Savio Polverari**, Montreal (CA); **Christopher Michael Lewis**, Vancouver, WA (US); **Matthew Gerard Fabian, Sr.**, Breezy Point, MN (US)

(73) Assignee: **Kemira Oyj** (FI)

(\*) Notice: Subject to any disclaimer, the term of this patent is extended or adjusted under 35 U.S.C. 154(b) by 512 days.

(21) Appl. No.: **11/531,911**

(22) Filed: **Sep. 14, 2006**

(65) **Prior Publication Data**

US 2008/0066880 A1 Mar. 20, 2008

(51) **Int. Cl.**

**D21H 21/10** (2006.01)  
**D21H 17/09** (2006.01)  
**D21H 17/10** (2006.01)  
**D21H 23/14** (2006.01)

(52) **U.S. Cl.** ..... **162/183**; 162/158; 162/164.1; 162/168.1; 162/168.2; 162/168.3; 162/181.6; 162/181.8

(58) **Field of Classification Search** ..... 162/158, 162/164.1, 168.1, 168.3, 164.6, 164.3, 183, 162/181.1, 181.2, 181.3, 181.8, 179, 181.6, 162/181.7

See application file for complete search history.

(56) **References Cited**

## U.S. PATENT DOCUMENTS

|             |         |                |
|-------------|---------|----------------|
| 4,021,364 A | 5/1977  | Speiser et al. |
| 4,913,775 A | 4/1990  | Langley et al. |
| 4,929,655 A | 5/1990  | Takeda et al.  |
| 4,968,435 A | 11/1990 | Neff et al.    |
| 5,006,590 A | 4/1991  | Takeda et al.  |

|              |           |                                 |
|--------------|-----------|---------------------------------|
| 5,006,890 A  | 4/1991    | Ishida et al.                   |
| 5,152,903 A  | 10/1992   | Neff et al.                     |
| 5,167,766 A  | 12/1992   | Honig et al.                    |
| 5,171,808 A  | 12/1992   | Ryles et al.                    |
| 5,274,055 A  | 12/1993   | Honig et al.                    |
| 5,340,865 A  | 8/1994    | Neff et al.                     |
| 5,389,203 A  | 2/1995    | Sawayama et al.                 |
| 5,393,381 A  | 2/1995    | Hund et al.                     |
| 5,431,783 A  | 7/1995    | Honig                           |
| 5,480,934 A  | 1/1996    | Messner et al.                  |
| 5,501,774 A  | 3/1996    | Burke                           |
| 5,597,858 A  | 1/1997    | Ramesh et al.                   |
| 5,597,859 A  | 1/1997    | Hurlock et al.                  |
| 5,882,525 A  | 3/1999    | Neff et al.                     |
| 5,958,188 A  | 9/1999    | Heard et al.                    |
| 6,007,679 A  | * 12/1999 | Nagarajan et al. .... 162/168.3 |
| 6,310,157 B1 | 10/2001   | Heard et al.                    |

(Continued)

## FOREIGN PATENT DOCUMENTS

EP 0462365 A1 3/1991

(Continued)

## OTHER PUBLICATIONS

Machine Translation of JP 2003-246909, published on Sep. 5, 2009.\*

(Continued)

Primary Examiner — José A Fortuna

(74) Attorney, Agent, or Firm — Cantor Colburn LLP

(57) **ABSTRACT**

According to the present invention, a process is provided for making paper or board comprising forming a cellulosic suspension that may or may not comprise a filler, flocculating the cellulosic suspension, draining the cellulosic suspension on a screen to form a sheet, wherein the cellulosic suspension is flocculated using a flocculation system comprising the sequential or simultaneous addition of a siliceous material and an organic, cationic or anionic, dispersion micropolymer in a salt solution.

**27 Claims, 5 Drawing Sheets**



## U.S. PATENT DOCUMENTS

|              |      |         |                                  |
|--------------|------|---------|----------------------------------|
| 6,391,156    | B1   | 5/2002  | Hjalmarson et al.                |
| 6,395,134    | B1 * | 5/2002  | Chen et al. .... 162/168.1       |
| 6,432,271    | B1 * | 8/2002  | Wong Shing et al. .... 162/168.3 |
| 6,454,902    | B1   | 9/2002  | Chen                             |
| 6,524,439    | B2   | 2/2003  | Chen et al.                      |
| 6,605,674    | B1   | 8/2003  | Whipple et al.                   |
| 6,616,806    | B2   | 9/2003  | I Chen                           |
| 7,250,448    | B2 * | 7/2007  | Walchuk et al. .... 516/20       |
| 7,507,781    | B2 * | 3/2009  | Walchuk et al. .... 526/81       |
| 2002/0066540 | A1 * | 6/2002  | Chen et al. .... 162/17          |
| 2004/0034145 | A1   | 2/2004  | Fischer et al.                   |
| 2006/0000568 | A1 * | 1/2006  | Polverari et al. .... 162/158    |
| 2006/0142430 | A1 * | 6/2006  | Harrington et al. .... 524/13    |
| 2006/0142431 | A1 * | 6/2006  | Sutman et al. .... 524/13        |
| 2006/0254464 | A1 * | 11/2006 | Nyander et al. .... 106/600      |
| 2006/0289136 | A1 * | 12/2006 | Doherty et al. .... 162/158      |
| 2006/0289137 | A1 * | 12/2006 | Gelman et al. .... 162/168.3     |
| 2008/0066880 | A1 * | 3/2008  | Polverari et al. .... 162/158    |
| 2008/0128102 | A1 * | 6/2008  | Polverari et al. .... 162/168.3  |
| 2009/0188640 | A1   | 7/2009  | Harrington                       |
| 2009/0211719 | A1 * | 8/2009  | Sutman et al. .... 162/164.6     |

## FOREIGN PATENT DOCUMENTS

|    |               |      |        |
|----|---------------|------|--------|
| EP | 0484617       | A1   | 4/1991 |
| JP | 2003246909    | A *  | 9/2003 |
| WO | 97/18351      |      | 5/1997 |
| WO | 98/24973      |      | 6/1998 |
| WO | 2004029360    | A1   | 4/2004 |
| WO | WO 2008033490 | A1 * | 3/2008 |

## OTHER PUBLICATIONS

European Patent Office, PCT International Search Report, International Application No. PCT/US2007/019976, Date of Mailing: Feb. 6, 2008.

European Patent Office, PCT Written Opinion of the ISA, International Application No. PCT/US2007/019976, Date of Mailing: Feb. 6, 2008.

JP2003246909; Publication Date: Sep. 5, 2003 (translation of abstract only).

Harris, Neil, et al. "Decoupling—The Latest Developments in Retention and Drainage Technology", African Pulp and Paper Week 2004; [http://www.tappa.co.za/archive2/APPW\\_2004>Title2004/Decoupling/decoupling.html](http://www.tappa.co.za/archive2/APPW_2004>Title2004/Decoupling/decoupling.html); Sep. 1, 2006.

EP 0624617, Publication date: Nov. 17, 1994, Abstract, 1 page.

EP 0664302, Publication date: Jul. 26, 1995, Abstract, 1 page.

EP 0674678, Publication date: Mar. 10, 1999, Abstract, 6 pages.

U.S. Appl. No. 11/855,475, filed Sep. 14, 2007.

JP1997078487A; Mar. 25, 1997; Machine Translation (9 pages).

JP1996059740A; Mar. 5, 1996; Machine Translation (27 pages).

JP1996060592A; Mar. 5, 1996; Machine Translation (20 pages).

U.S. Appl. No. 11/855,475 Non-Final Office Action dated: Jan. 12, 2009, 69 pages.

U.S. Appl. No. 11/855,475 Final Office Action dated: Sep. 1, 2009, 8 pages.

U.S. Appl. No. 11/855,475 Advisory Action dated: Aug. 19, 2010, 3 pages.

U.S. Appl. No. 11/855,475 Final Office Action dated: Jun. 7, 2010, 7 pages.

U.S. Appl. No. 11/855,475 Non-Final Office Action dated: Nov. 10, 2009, 11 pages.

\* cited by examiner

Figure 1



Figure 2



Figure 3



Figure 4



Figure 5



Figure 6



Figure 7



Figure 8



## METHOD FOR PAPER PROCESSING

## BACKGROUND OF INVENTION

This invention relates to processes for making paper and paperboard from a cellulosic stock, employing a novel flocculation system in which a new micropolymer technology is employed.

During the manufacture of paper and paperboard, a cellulosic thin stock is drained on a moving screen (often referred to as a machine wire) to form a sheet, which is then dried. It is well known to apply water-soluble polymers to the cellulosic suspension in order to effect flocculation of the cellulosic solids and enhance drainage on the moving screen.

In order to increase output of paper, many modern papermaking machines operate at higher speeds. As a consequence of increased machine speeds, a great deal of emphasis has been placed on drainage and retention systems that provide increased drainage and retention of the papermaking components. It is known that increasing the molecular weight of a polymeric retention aid (which is generally added immediately prior to drainage) will tend to increase the rate of drainage, but will also damage formation. It is difficult to obtain the optimum balance of retention, drainage, drying and formation by adding a single polymeric retention aid, and it is therefore common practice to add two separate materials in sequence.

U.S. Pat. No. 4,913,775 provides a process wherein paper or paperboard is made by forming an aqueous cellulosic suspension, passing the suspension through one or more shear stages selected from cleaning, mixing and pumping, draining the suspension to form a sheet, and drying the sheet. The suspension that is drained includes an organic polymeric material that is a flocculant or a retention aid, and an inorganic material comprising bentonite, which is added in an amount of at least 0.03% to the suspension after one of the shear stages. The organic polymeric retention aid or flocculant comprises a substantially linear synthetic cationic polymer having molecular weight above 500,000 and having a charge density of at least about 0.2 equivalents of nitrogen per kilogram of polymer. The organic polymeric retention aid or flocculant is added to the suspension before the shear stage in an amount such that flocs are formed. The flocs are broken by the shearing to form microflocs that resist further degradation by the shearing, and that carry sufficient cationic charge to interact with the bentonite to give better retention than that which is obtainable when adding the polymer alone after the last point of high shear. This process is commercialized by Ciba Specialty Chemicals under the "Hydrocol O" trademark.

More recent attempts to improve drainage and retention during papermaking have used variations on this theme by using different polymers, siliceous components and more than two components.

U.S. Pat. No. 4,968,435 describes a method of flocculating an aqueous dispersion of suspended solids which comprises adding to, and mixing with the dispersion, from about 0.1 to about 50,000 parts per million of dispersion, solids of an aqueous solution of a water-insoluble, crosslinked, cationic, polymeric flocculant having an unswollen number average particle size diameter of less than about 0.5 micrometers, a solution viscosity of about 1.2 to about 1.8 centipoise, and a crosslinking agent content above about 4 molar parts per million, based on the monomeric units present in the polymer, to flocculate the suspended solids, and separating the flocculated suspended solids from the dispersion.

U.S. Pat. No. 5,152,903 is a continuation of this patent, and describes a method of flocculating a dispersion of suspended solids that comprises adding to, and mixing with the dispersion, from about 0.1 to about 50,000 parts per million of dispersion solids of an aqueous solution of a water-soluble, crosslinked, cationic, polymeric flocculant having an unswollen number average particle size diameter of less than about 0.5 micrometers, a solution viscosity of from about 1.2 to about 1.8 centipoise and a crosslinking agent content above about 4 molar parts per million based on the monomeric units present in the polymer.

U.S. Pat. No. 5,167,766 further describes a method of making paper which comprises adding to an aqueous paper furnish from about 0.05 to about 20 pounds per ton, based on the dry weight of paper furnish solids, of an ionic, organic, crosslinked polymeric microbead, the microbead having an unswollen particle diameter of less than about 750 nanometers and an ionicity of at least 1%, but at least 5%, if anionic and used alone.

U.S. Pat. No. 5,171,808 is a further example which describes a composition comprising crosslinked anionic or amphoteric polymeric micropolymers derived solely from the polymerization of an aqueous solution of at least one monomer, the micropolymers having an unswollen number average particle size diameter of less than about 0.75 micrometers, a solution viscosity of at least about 1.1 centipoise, a crosslinking agent content of about 4 molar parts to about 4000 parts per million, based on the monomeric units present in the polymer, and an ionicity of at least about 5 mole percent.

U.S. Pat. No. 5,274,055 describes a papermaking process wherein improved drainage and retention are obtained when ionic, organic microbeads, of less than about 1,000 nanometers in diameter if crosslinked or less than about 60 nanometers in diameter if non crosslinked, are added either alone or in combination with a high molecular weight organic polymer and/or polysaccharide. Further addition of alum enhances drainage formation and retention properties in papermaking stock with and without the presence of other additives used in papermaking processes.

U.S. Pat. No. 5,340,865 describes a flocculant comprising a water-in-oil emulsion comprising an oil phase and an aqueous phase wherein the oil phase consists of fuel oil, kerosene, odorless mineral spirits or mixtures thereof, and one more surfactants at an overall HLB ranging from about 8 to 11, wherein the aqueous phase is in the form of micelles and contains a crosslinked, cationic, polymer produced from about 40 to about 99 parts by weight of acrylamide and about 1 to about 60 parts by weight of a cationic monomer selected from N,N-dialkylaminoalkylacrylates and methacrylates, and their quaternary or acid salts, N,N-dialkylaminoalkylacrylamides and methacrylamides, and their quaternary or acid salts, and diallyldimethylammonium salts. The micelles have a diameter of less than about 0.1 micrometers, and the polymer has a solution viscosity of from about 1.2 to about 1.8 centipoise, and a content of N,N-methylenebisacrylamide of about 10 molar parts to about 1000 molar parts per million, based on the monomeric units present in the polymer.

U.S. Pat. No. 5,393,381 describes a process of making paper or board by adding a water-soluble branched cationic polyacrylamide and a bentonite to the fibrous suspension of pulp. The branched cationic polyacrylamide is prepared by polymerizing a mixture of acrylamide, cationic monomer, branching agent, and chain transfer agent by solution polymerization.

U.S. Pat. No. 5,431,783 describes a method for providing improved liquid-solid separation performance in liquid par-

ticulate dispersion systems. The method comprising adding to a liquid system containing a plurality of finely divided particles from about 0.05 to about 10 pounds per ton, based upon the dry weight of the particles, of an ionic, organic crosslinked polymeric microbead with a diameter of less than about 500 nanometers, and from about 0.05 to about 20 pounds per ton, on the same basis, of a polymeric material selected from the group consisting of polyethylenimines, modified polyethylenimines, and mixtures thereof. In addition to the compositions described above, additives such as organic ionic polysaccharides may also be combined with the liquid system to facilitate separation of the particulate material therefrom.

U.S. Pat. No. 5,501,774 describes a process where filled paper is made by providing an aqueous feed suspension containing filler and cellulosic fiber, coagulating the fiber and filler in the suspension by adding cationic coagulating agent, making an aqueous thinstock suspension by diluting a thickstock consisting of or formed from the coagulated feed suspension, adding anionic particulate material to the thinstock or to the thickstock from which the thinstock is formed, subsequently adding polymeric retention aid to the thinstock and draining the thinstock for form a sheet and drying the sheet.

U.S. Pat. No. 5,882,525 describes a process in which a cationic branched water-soluble polymer with a solubility quotient greater than about 30% is applied to a dispersion of suspended solids, e.g. a paper making stock, in order to release water. The cationic, branched, water-soluble polymer is prepared from similar ingredients to U.S. Pat. No. 5,393,381, by polymerizing a mixture of acrylamide, cationic monomer, branching agent and chain transfer agent.

U.S. Pat. No. 5,958,188 further describes a process where paper is made by a dual soluble polymer process in which a cellulosic suspension, which usually contains alum or cationic coagulant, is first flocculated with a high intrinsic viscosity cationic synthetic polymer or cationic starch and, after shearing, the suspension is reflocculated by the addition of a branched anionic water-soluble polymer having an intrinsic viscosity above 3 deciliters per gram, and a tan delta at 0.005 Hertz of at least 0.5.

U.S. Pat. No. 6,454,902 describes a process for making paper comprising forming a cellulosic suspension, flocculating the suspension, draining the suspension on a screen to form a sheet, and then drying the sheet, wherein the cellulosic suspension is flocculated by addition of a polysaccharide or a synthetic polymer of intrinsic viscosity at least 4 deciliters per gram, and then reflocculated by a subsequent addition of a reflocculating system, wherein the reflocculation system comprises a siliceous material and a water-soluble polymer. In one embodiment, the siliceous material is added prior to or simultaneously with the water-soluble polymer. In another embodiment, the water-soluble polymer is anionic and added prior to the siliceous material.

U.S. Pat. No. 6,524,439 provides a process for making paper or paperboard comprising forming a cellulosic suspension, flocculating the suspension, draining the suspension on a screen to form a sheet and then drying the sheet. The process is characterized in that the suspension is flocculated using a flocculation system comprising a siliceous material and organic microparticles that have an unswollen particle diameter of less than 750 nanometers.

JP Publication No. 2003-246909 discloses polymer dispersions is produced by combining an amphoteric polymer having a specific cationic structural unit and an anionic structural unit and soluble in the salt solution, and a specific anionic

polymer soluble in the salt solution and polymerizing them in dispersion under agitation in the salt solution.

However, there still exists a need to further enhance paper making processes by further improving drainage, retention and formation. Furthermore there also exists the need for providing a more effective flocculation system for making highly filled paper.

## SUMMARY

The above-described drawbacks and disadvantages are alleviated by a process for making paper or paperboard, comprising: forming a cellulosic suspension; flocculating the cellulosic suspension; draining the cellulosic suspension on a screen to form a sheet; and drying the sheet; wherein the cellulosic suspension is flocculated by adding a flocculation system comprising a siliceous material and an organic, anionic or cationic, dispersion micropolymer in a salt solution, wherein the siliceous material and the organic micropolymer are added simultaneously or sequentially.

In another embodiment, a paper or paperboard is provided, made by the above process.

Further advantages of the invention are described in the following Figures and Detailed Description.

## BRIEF DESCRIPTION OF THE FIGURES

FIG. 1 is a schematic diagram illustrating where the components of the flocculating systems can be added in the paper and paperboard making process.

FIG. 2 is a graph of the retention data of Example 1 for a furnish that does not contain wood.

FIG. 3 is a graph of the retention data of Example 2 for a furnish that does not contain wood.

FIG. 4 is a graph of the retention data of Example 3 for a wood-containing furnish for super calendered grades.

FIG. 5 is a graph of the drainage response via a dynamic drainage analyzer with recirculation for a wood-containing furnish for super calendered grades as in Example 3.

FIG. 6 is a graph of the drainage response under vacuum in a single pass for a wood-containing furnish for super calendered grades as in Example 3.

FIG. 7 is the graph of the drainage response and retention response in a single pass for Example 4.

FIG. 8 is the graph of the drainage response and retention response in a single pass for Example 5.

## DETAILED DESCRIPTION

The inventors hereof have unexpectedly discovered that in the manufacture of paper or paperboard products, flocculation is significantly improved by use of an organic, cationic or anionic, micropolymer salt solution in combination with a siliceous material. Use of this flocculation system provides improvements in retention, drainage, and formation compared to a system using the organic micropolymer alone, or the siliceous material in the absence of the organic micropolymer.

Thus, in accordance with the present disclosure, a process is provided for making paper or paperboard, comprising forming a cellulosic suspension, flocculating the cellulosic suspension, draining the cellulosic suspension on a screen to form a sheet, and then drying the sheet, wherein the cellulosic suspension is flocculated by adding a flocculation system comprising an organic, anionic or cationic, micropolymer in a salt solution and a siliceous material, added simultaneously or sequentially.

In an specific exemplary embodiment, the process by which paper or paperboard is made comprises forming an aqueous cellulosic suspension, passing the aqueous cellulosic suspension through one or more shear stages selected from cleaning, mixing, pumping, and combinations thereof, draining the cellulosic suspension to form a sheet, and drying the sheet. The drained cellulosic suspension used to form the sheet comprises a cellulosic suspension that is flocculated with an organic micropolymer and an inorganic siliceous material, which are added, simultaneously or sequentially, in an amount of at least about 0.01 percent by weight, based on the total weight of the dry cellulosic suspension, to the cellulosic suspension after one of the shear stages. In addition, the drained cellulosic suspension used to form the sheet comprises an organic polymeric retention aid or flocculant comprising a substantially linear synthetic cationic, non ionic, or anionic polymer having a molecular weight greater than or equal to about 500,000 atomic mass units that is added to the cellulosic suspension before the shear stage in an amount such that flocs are formed by the addition of the polymer, and the flocs are broken by the shearing to form microflocs that resist further degradation by the shearing and that carry sufficient anionic or cationic charge to interact with the siliceous material and organic micropolymer to give better retention than the retention that is obtainable when adding the organic micropolymer alone after the last point of high shear.

In some embodiments, one or more shear stages comprise a centriscreen. The polymer is added to the cellulosic suspension before the centriscreen, and the flocculation system (micropolymer/siliceous material) is added after the centriscreen.

At a minimum, the flocculation system disclosed herein comprises an organic, anionic or cationic, micropolymer salt solution in combination with a siliceous material. The organic micropolymer is in the form of an aqueous salt solution and is a mixture of linear polymers and/or long chain branched polymers. The aqueous salt solution of the organic micropolymer mixture has a reduced specific viscosity above 0.2 deciliters per gram (dl/g). Suitable micropolymers can be prepared by initiating polymerization of an aqueous mixture of monomers in a salt solution to form a organic micropolymer. The monomers are selected from the group consisting of acrylamide, methacrylamide, diallyldimethylammonium chloride, dimethylaminoethyl acrylate methyl chloride quaternary salt, dimethylaminoethyl methacrylate methyl chloride quaternary salt, acrylamidopropyltrimethylammonium chloride, methacrylamidopropyltrimethylammonium chloride, acrylic acid, sodium acrylate, methacrylic acid, sodium methacrylate, ammonium methacrylate, and the like, and a combination comprising at least one of the foregoing monomers.

In particular, a dispersion of the organic micropolymer is prepared by polymerizing the monomer mixture containing at least 2 mole percent of a cationic or anionic monomer in an aqueous solution of a polyvalent ionic salt. The polymerization is carried out in an aqueous solution comprising about 1 to about 10 percent by weight, based on the total weight of the monomers, of a dispersant polymer, the dispersant polymer being a water-soluble anionic or cationic polymer which is soluble in the aqueous solution of the polyvalent anionic salt. The polyvalent ionic salt comprises phosphates, sulfates, and combinations thereof. The organic micropolymers exhibit a solution viscosity of greater than or equal to about 0.5 centipoise (millipascal-second) and have an ionicity of greater than or equal to about 5.0 percent.

The siliceous material is an anionic microparticulate or nanoparticulate silica-based material. The siliceous material

is selected from the group consisting of hectorite, smectites, montmorillonites, nontronites, saponite, saucnite, hormites, attapulgites, laponite, sepiolites, and the like. Combinations comprising at least one of the foregoing siliceous materials can be used. The siliceous material also can be any of the materials selected from the group consisting of silica based particles, silica microgels, colloidal silica, silica sols, silica gels, polysilicates, aluminosilicates, polyaluminosilicates, borosilicates, polyborosilicates, zeolites, swellable clay, and the like, and a combination of at least one of the foregoing siliceous materials. Bentonite-type clays can be used. The bentonite can be provided as an alkali metal bentonite, either in powder or slurry form. Bentonites occur naturally either as alkaline bentonites, such as sodium bentonite, or as the alkaline earth metal salt, such as the calcium or magnesium salt.

These components of the flocculation system are introduced into the cellulosic suspension either sequentially or simultaneously. Preferably, the siliceous material and the polymeric micropolymers are introduced simultaneously. When introduced simultaneously, the components can be kept separate before addition, or can be premixed. When introduced sequentially, the organic micropolymer is introduced into the cellulosic suspension before the siliceous material.

In another embodiment, the flocculation system comprises three components, wherein the cellulosic suspension is pretreated by inclusion of a flocculant prior to introducing the organic micropolymer and siliceous material. The pretreatment flocculant can be anionic, nonionic, or cationic. It can be a synthetic or natural polymer, specifically a water-soluble, substantially linear or branched, organic polymer. The water-soluble organic polymers can be a natural polymer, such as cationic starch or synthetic cationic polymers such as polyamines, poly(diallyldimethylammonium chloride), polyamido amines, and polyethyleneimine. The pretreatment flocculant can also be a crosslinked polymer, or a blend of a crosslinked polymer and a water-soluble polymer. The pretreatment flocculant can also be an inorganic material such as alum, aluminum sulfate, polyaluminum chloride, aluminum chloride trihydrate and aluminum chlorohydrate, and the like.

Thus, in a specific embodiment of the paper or paperboard manufacturing process, the cellulosic suspension is first flocculated by introducing the pretreatment flocculent, then optionally subjected to mechanical shear, and then reflocculated by introducing the organic micropolymer and siliceous material simultaneously. Alternatively, the cellulosic suspension is reflocculated by introducing the siliceous material and then the organic micropolymer, or by introducing the organic micropolymer and then the siliceous material.

The pretreatment comprises incorporating the pretreatment flocculant into the cellulosic suspension at any point prior to the addition of the organic micropolymer and siliceous material. It can be advantageous to add the pretreatment flocculant before one of the mixing, screening or cleaning stages, and in some instances before the stock cellulosic suspension is diluted. It can even be advantageous to add the pretreatment flocculant into the mixing chest or blend chest or even into one or more of the components of the cellulosic suspension, such as coated broke, or filler suspensions, such as precipitated calcium carbonate slurries.

In still another embodiment, the flocculation system comprises four flocculent components, the organic micropolymer and siliceous material, a flocculant as described above, for example a water-soluble cationic flocculent, and an additional flocculent/coagulant that is an nonionic, anionic, or cationic water soluble polymer.

In this embodiment, the water soluble cationic flocculant can be organic, for example, water-soluble, substantially linear or branched polymers, either natural (e.g., cationic starch) or synthetic (e.g., polyamines, poly(diallyldimethylammonium chloride)s, polyamido amines, and poly(ethylene-imines). The water-soluble cationic flocculant can alternatively be an inorganic material such as alum, aluminum sulfate, polyaluminum chloride, aluminum chloride trihydrate and aluminum chlorohydrate, and the like. The water-soluble cationic flocculant is advantageously a water-soluble polymer, which can, for instance, be a relatively low molecular weight polymer of relatively high cationicity.

The at least one additional flocculant/coagulant is a water soluble polymer. The additional flocculant/coagulant component is preferably added prior to either the siliceous material, polymeric micropolymer or flocculating material. Typically the additional flocculent is a natural or synthetic polymer or other material capable of causing flocculation/coagulation of the fibres and other components of the cellulosic suspension. The additional flocculant/coagulant may be a cationic, non-ionic, anionic or amphoteric natural or synthetic polymer. It may natural polymer such as natural starch, cationic starch, anionic starch or amphoteric starch. Alternatively it may be any water soluble synthetic polymer which preferably exhibits its ionic character. The preferred ionic water soluble polymers have cationic or potentially cationic functionality. For instance the cationic polymer may comprise free amine groups which become cationic once introduced into a cellulosic suspension with a sufficiently low pH so as to protonate free amine groups. Preferably however, the cationic polymers carry a permanent cationic charge, such as quaternary ammonium groups. When anionic or cationic, the anionic or cationic polymer is formed from a water soluble ethylenically unsaturated monomer or water soluble blend of ethylenically unsaturated monomers comprising at least one anionic or cationic monomer. The cationic or anionic polymer is a branched or linear polymer which has an intrinsic viscosity above 2 dl/g. For instance, the polymer can be a homopolymer of any suitable ethylenically unsaturated cationic monomers.

Cationic flocculant/coagulants are desirably a water soluble polymer, which can, for instance be a relatively low molecular weight polymer of relatively high cationicity. For instance, the polymer can be a homopolymer of diallyl dimethyl ammonium chloride are exemplary. The low molecular weight, high cationicity polymers can be addition polymers formed by condensation of amines with other suitable di- or trifunctional species. For example, the polymer can be formed by reacting one or more amines selected from dimethyl amine, trimethyl amine, ethylene diamine, epihalohydrin, epichlorohydrin, and the like, and a combination of at least one of the foregoing amines. It is advantageous for the cationic flocculant/coagulant to be a polymer that is formed from a water-soluble ethylenically unsaturated cationic monomer or blend of monomers wherein at least one of the monomers in the blend is cationic or potentially cationic. A water-soluble monomer is a monomer having a solubility of at least 5 grams per 100 cubic centimeters of water. The cationic monomer is advantageously selected from diallyl dialkyl ammonium chlorides, acid addition salts or quaternary ammonium salts of either dialkyl aminoalkyl (meth) acrylate or dialkyl amino alkyl (meth)acrylamides. The cationic monomer can be polymerized alone or copolymerized with water-soluble non-ionic, cationic, or anionic monomers. It is advantageous for such polymers to have an intrinsic viscosity of at least 3 deciliters per gram. Specifically, up to about 18 deciliters per gram. More specifically, from about 7

up to about 15 deciliters per gram. The water-soluble cationic polymer can also have a slightly branched structure by incorporating up to about 20 parts per million by weight of a branching agent.

5 The additional flocculant/coagulant component is preferably added prior to either the siliceous material, organic micropolymer, or water soluble cationic flocculant.

In use, all of the components of the flocculation system can be added prior to a shear stage. It is advantageous for the last 10 component of the flocculation system to be added to the cellulosic suspension at a point in the process where there is no substantial shearing before draining to form the sheet. Thus it is advantageous that at least one component of the flocculation system is added to the cellulosic suspension, and the flocculated cellulosic suspension is then subjected to mechanical shear wherein the flocs are mechanically degraded and then at least one component of the flocculation system is added to reflocculate the cellulosic suspension prior 15 to draining.

In an exemplary embodiment, the first water-soluble cationic flocculant polymer is added to the cellulosic suspension and then the cellulosic suspension is mechanically sheared. The additional, higher molecular weight coagulant/flocculant 20 can then be added and then the cellulosic suspension is sheared through a second shear point. The siliceous material and the organic micropolymer are added last to the cellulosic suspension.

The organic micropolymer and siliceous material can be 25 added either as a premixed composition or separately but simultaneously, but they are advantageously added sequentially. Thus, the cellulosic suspension can be reflocculated by addition of the organic micropolymer followed by the siliceous material, but preferably the cellulosic suspension is reflocculated by adding siliceous material, and then the organic micropolymer.

The first component of the flocculation system can be 30 added to the cellulosic suspension and then the flocculated cellulosic suspension can be passed through one or more shear stages. The second component of the flocculation system can be added to reflocculate the cellulosic suspension, and then the reflocculated suspension can be subjected to further mechanical shearing. The sheared reflocculated cellulosic suspension can also be further flocculated by addition 35 of a third component of the flocculation system. In the case where the addition of the components of the flocculation system is separated by shear stages, it is advantageous that the organic micropolymer and the siliceous material are the last components to be added, at a point in the process where there 40 will no longer be any shear.

In another embodiment, the cellulosic suspension is not 45 subjected to any substantial shearing after addition of any of the components of the flocculation system to the cellulosic suspension. The siliceous material, organic micropolymer, and optionally, the coagulating material, can all be introduced into the cellulosic suspension after the last shear stage prior to draining. In such embodiments, the organic micropolymer can be the first component followed by either the coagulating material (if included), and then the siliceous material. However, other orders of addition can also be used, with all the 50 components or just the siliceous material and the organic micropolymer being added.

FIG. 1 is a schematic diagram illustrating the various 55 points in the papermaking process where the additional flocculant/coagulant ("A" in diagram), the pretreatment coagulant and the cationic water-soluble coagulant ("B" in dia-

gram), the organic micropolymer ("C" in diagram) and the siliceous material ("D" in diagram) can be added during the process.

Suitable amounts of each of the components of the flocculation system will depend on the particular component, the composition of the paper or paperboard being manufactured, and like considerations, and are readily determined without undue experimentation in view of the following guidelines. In general, the amount of siliceous material is about 0.05 to about 5.0 kg per metric ton (kg/MT); the amount of organic micropolymer dispersion is about 0.05 to about 3.0 kg/MT; and the amount of any one of the coagulants and coagulant/dispersant is about 0.05 to about 10.0 kg/MT. It is to be understood that these amounts are guidelines, but are not limiting, due to different types and amounts of actives in the solutions or dispersions:

The process disclosed herein can be used for making filled paper. The paper making stock comprises any suitable amount of filler. In some embodiments, the cellulosic suspension comprises up to about 50 percent by weight of a filler, generally about 5 to about 50 percent by weight of filler, specifically about 10 to about 40 percent by weight of filler, based on the dry weight of the cellulosic suspension. Exemplary fillers include precipitated calcium carbonate, ground calcium carbonate, kaolin, calcium sulphite, titanium dioxide, and the like, and a combination comprising at least one of the foregoing fillers. Thus, according to this embodiment, a process is provided for making filled paper or paperboard; wherein a cellulosic suspension comprises a filler, and wherein the cellulosic suspension is flocculated by introducing a flocculation system comprising a siliceous material and an organic micropolymer as described previously. In other embodiments, the cellulosic suspension is free of a filler.

The invention is further illustrated by the following non-limiting examples. The components used in the examples are listed in Table 1.

TABLE 1

| Abbreviation | Component                                                                                                                                                                                                                |
|--------------|--------------------------------------------------------------------------------------------------------------------------------------------------------------------------------------------------------------------------|
| PAM          | Polyacrylamide flocculant                                                                                                                                                                                                |
| A-Pam        | Anionic polyacrylamide flocculant                                                                                                                                                                                        |
| ANNP         | Colloidal silica                                                                                                                                                                                                         |
| ANMP         | Anionic micropolymer synthesized in a salt solution comprising acrylamide monomers and acrylic acid, having about 30 mole percent anionic charge, and an average molecular mass of about 5 MM Daltons.                   |
| ANMPP        | Crosslinked micropolymer that is not polymerized in a salt solution, and is in an oil and water system                                                                                                                   |
| P-6,524,439  | ANMPP with colloidal silica as described in U.S. Pat. No. 6,524,439                                                                                                                                                      |
| C-Pam        | Linear cationic polyacrylamide flocculant                                                                                                                                                                                |
| CatMP        | Cationic micropolymer, comprising acrylamide and N,N-dimethylaminopropyl acrylamide units, having about 25 mole percent cationic charge, and an average molecular mass of about 5 MM Daltons.                            |
| P-4,913,775  | Linear cationic polyacrylamide C-Pam with bentonite as described in U.S. Pat. No. 4,913,775                                                                                                                              |
| PAC          | Polyaluminum chloride coagulant                                                                                                                                                                                          |
| DDA          | Dynamic drainage analyzer                                                                                                                                                                                                |
| VDT          | Vacuum drainage tester                                                                                                                                                                                                   |
| CatMP-SS     | Cationic micropolymer dispersion in a salt solution, comprising acrylamide and 2-(dimethylamino)ethyl acrylate units, having about 10 mole percent cationic charge, and an average molecular mass of about 7 MM Daltons. |
| IMP-L        | Laponite, an inorganic, hydrated, microparticulate silicate.                                                                                                                                                             |

## EXAMPLE 1

The following example illustrates the advantages of using a combination of a siliceous material and a dispersion

micropolymer in a salt solution in paper production. The siliceous material is ANNP, and the dispersion micropolymer in a salt solution is ANMP. The data is from a study done with a 100 percent wood-free uncoated free sheet furnish under alkaline conditions. The furnish contains precipitated calcium carbonate (PCC) filler at a level of 29 percent by weight, based on the total weight of the furnish. Table 1 displays a list of the abbreviations used below.

The retention data are expressed in FIG. 1 as the percent improvements observed over a non-treated system for the retention parameters of first pass solids retention (FPR), and first pass ash retention (FPAR). For the no PAM portion of the study, a clear increase in efficiency is observed when both the ANMP and the ANNP are applied together. The improved performance is particularly evident at the lower application rates for these components. A similar response is observed for the portion of the evaluation that included the application of A-Pam. Again, the combination of the ANMP and the ANNP in the presence of A-Pam maximizes the retention response for both ash and total solids. Moreover, the data show that with the ANMP and ANNP combination program, the level of A-Pam required to get a desired level of retention of total solids or ash is significantly lower than with either single application of ANMP or ANNP. Lower levels of A-Pam are desirable when trying to increase retention as this will minimize the negative impact on formation. This is a primary quality goal of the finished paper/paperboard products.

## EXAMPLE 2

The following example illustrates the advantage of applying a dispersion micropolymer in a salt solution with colloidal silica, in the presence of anionic polyacrylamide over the application of an oil in water emulsion micropolymer with colloidal silica in the presence of anionic polyacrylamide per the application described by U.S. Pat. No. 6,524,439. The data is from a study done with a 100 percent wood-free, uncoated, free sheet furnish under alkaline conditions. The furnish contains PCC filler at a level of 13 percent by weight.

The data in FIG. 2 show that the highest retention response is achieved with the salt-based micropolymer and colloidal silica application. The retention efficiency of this chemistry is greater than the crosslinked oil and water emulsion application described per U.S. Pat. No. 6,524,439.

## EXAMPLE 3

The following data is from a study done with a wood containing furnish comprising 70 percent by weight thermomechanical pulp (TMP), 15 percent by weight ground wood pulp, and 15 percent by weight bleached kraft pulp used for super calendered (SC) paper production in alkaline conditions. The furnish contains PCC filler at a level of 28 percent by weight.

The results of this study show both retention and drainage rate data. Retention data are displayed in FIG. 3, while drainage rate data are displayed in FIG. 4 and FIG. 5. The data deal with PAC and C-Pam with a CatMP produced by polymerizing a monomer mixture containing a cationic monomer in an aqueous solution of a polyvalent salt applied with ANNP, PAC and C-Pam with ANMP produced by polymerizing a monomer mixture containing an anionic monomer in an aqueous solution of a polyvalent anionic salt applied with ANNP, and C-Pam with a swellable mineral as described in U.S. Pat. No. 6,524,439.

The retention data in FIG. 3 illustrate the improved performance of the application using catMP applied with ANNP in

## 11

the presence of C-Pam over the application using bentonite and C-Pam according to U.S. Pat. No. 6,524,439. Moreover, the application using ANMP with ANNP in the presence of C-Pam is superior to the applications including the application under U.S. Pat. No. 6,524,439.

FIG. 4 shows the results from a drainage evaluation using a DDA where the filtrate is recirculated and used for subsequent iterations. This gives a close simulation to the fully scaled up process. In this study, the number of recirculations was 4. Parameters shown are drainage time and sheet permeability. FIG. 4 illustrates the increased performance achieved over an ANMP application alone in the presence of C-Pam and PAC when the ANMP is applied in conjunction with the ANNP, in the presence of C-Pam and PAC. The drainage performance of the ANMP/ANNP program is greater than the bentonite C-Pam application as described by U.S. Pat. No. 6,524,439. This is desirable on paper machines where furnish drainage limits production rate.

FIG. 5 depicts similar results to that observed in FIG. 4. FIG. 5 shows the drainage response results for a study using a VDT. This is a single pass test and similarly to the DDA, determines drainage time rate and sheet permeability. The ANMP applied in conjunction with ANNP in the presence of PAC and C-Pam gives the highest drainage rate. This rate is greater than that achieved by a swellable mineral application using bentonite per the application as described U.S. Pat. No. 6,524,439.

## EXAMPLE 4

The following example illustrates the enhanced performance in the paper and board making process when the dispersion micropolymer in a salt solution is applied, alone or in combination with siliceous material, compared to when C-Pam is applied, alone or in combination with a siliceous material. The data is from a study done on wood containing furnish used for newsprint production under acidic conditions. The furnish comprises about 5 percent by weight ash, predominantly kaolin. The dispersion micropolymer in a salt solution is CatMP-SS.

The drainage response was measured with a modified Schopper Reigler drainage tester using a single pass, while the retention characteristics were determined using a dynamic drainage jar. The results of this study are depicted in FIG. 6.

The data in FIG. 6 illustrate the enhanced performance in the paper and board making process when CatMP-SS is applied, alone or in combination with ANNP, compared to when C-Pam is applied, alone or in combination with ANNP. An improvement in both the drainage and retention rates are observed. The data also indicate that it is advantageous to apply the CatMP-SS before a point of shear. Not wishing to be bound by any particular theory, it is believed that the improvement observed is due to the high degree of branching and charge within the CatMP-SS compared to polymers used in the art. When the CatMP-SS is sheared, the result is a higher degree of charge, an effect referred to as the ionic regain of a polymer. The data suggests that the CatMP-SS is giving ionic regain values greater than 100%, which is not possible when using a linear cationic polyacrylamide such as C-Pam. The ionic regain promotes reactivity with the siliceous material, such as ANNP, the latter not being very efficient under acidic conditions as known in the art. According to the data in FIG. 6, when ANNP is added to C-Pam, the net improvement in the drainage and retention response is negligible. On the other

## 12

hand, when ANNP is added to CatMP-SS, the drainage and retention response is improved by over 20%.

## EXAMPLE 5

5 The following example illustrates the advantages gained when the siliceous material is used in combination with the dispersion micropolymer in salt solution under acidic conditions, when compared to the use of the siliceous material in 10 combination with regular polymers used in the art under acidic conditions. The data is from a study done on wood containing furnish used for newsprint production under acidic conditions. The furnish comprises about 5 percent by weight ash, predominantly kaolin. The drainage retention and 15 response were measured as discussed above.

The results are presented in FIG. 7. As expected, U.S. Pat. 20 No. 4,913,775 shows that it is advantageous to add bentonite to C-Pam as opposed to adding ANNP or IMP-L to C-Pam, because the system is under acidic conditions. However, 25 when CatMP-SS is added to the combination of C-Pam and the siliceous material, the drainage performance is enhanced by more than 30% for the IMP-L system and more than 40% for the ANNP system. The combination of CatMP-SS with C-Pam and the siliceous material outperforms the combination of C-Pam and the siliceous material without CatMP-SS as per U.S. Pat. No. 4,913,775. This result highlights the 30 advantages of CatMP-SS as discussed in Example 4.

The terms "a" and "an" do not denote a limitation of quantity, but rather denote the presence of at least one of the 35 referenced item. The term "water-soluble" refers to a solubility of at least 5 grams per 100 cubic centimeters of water. All cited patents, patent applications, and other references are incorporated herein by reference in their entirety as though set forth in full.

35 While the invention has been described with reference to some embodiments, it will be understood by those skilled in the art that various changes can be made and equivalents can be substituted for elements thereof without departing from the scope of the invention. In addition, many modifications can be made to adapt a particular situation or material to the 40 teachings of the invention without departing from essential scope thereof. Therefore, it is intended that the invention not be limited to the particular embodiments disclosed as the best mode contemplated for carrying out this invention, but that the invention will include all embodiments falling within the 45 scope of the appended claims.

What is claimed is:

1. A process for making paper or paperboard, comprising: forming a cellulosic suspension; passing the cellulosic suspension through one or more shear stages; draining the cellulosic suspension on a screen to form a sheet; and drying the sheet; wherein the cellulosic suspension is flocculated before draining by adding a flocculation system comprising greater than or equal to about 0.01 percent by weight of an organic micropolymer in a salt solution; and an inorganic siliceous material; wherein the organic micropolymer and the inorganic siliceous material are added after one of the shear stages; wherein the organic micropolymer and the inorganic siliceous material are added simultaneously or sequentially; wherein the flocculation system further comprises an organic water-soluble flocculant material comprising a substantially linear synthetic cationic, non-ionic, or anionic polymer, having molecular weight greater than

## 13

or equal to about 500,000 atomic mass units, that is added to the cellulosic suspension before the shear stage in an amount such that flocs are formed; wherein the flocs are broken by the shearing to form microflocs that resist further degradation by the shearing, and that carry sufficient anionic or cationic charge to interact with the siliceous material and the organic micropolymer to give better retention than that which is obtained when adding the flocculation system after the last point of high shear without first adding the flocculant material to the cellulosic suspension; wherein percent by weight is based on the total weight of the dry cellulosic suspension.

2. The process of claim 1, wherein the organic micropolymer is part of a salt solution prepared by initiating polymerization of an aqueous mixture of a monomer in a salt solution to form an organic micropolymer dispersion, having a reduced specific viscosity greater than or equal to about 0.2 deciliters per gram.

3. The process of claim 2, wherein the monomer is acrylamide, methacrylamide, diallyldimethylammonium chloride, dimethylaminoethyl acrylate methyl chloride quaternary salt, dimethylaminoethyl methacrylate methyl chloride quaternary salt, acrylamidopropyltrimethylammonium chloride, methacrylamidopropyltrimethylammonium chloride, acrylic acid, methacrylic acid, sodium acrylate, sodium methacrylate, ammonium methacrylate, or a combination comprising at least one of the foregoing monomers.

4. The process of claim 2, wherein the monomer comprises greater than or equal to about 2 mole percent of a cationic or anionic monomer, based on the total number of moles of monomer.

5. The process of claim 2, wherein the salt solution is an aqueous solution of a polyvalent ionic salt, and wherein the mixture of monomers in a salt solution comprises about 1 to about 10 percent by weight, based on the total weight of the monomers, a dispersant polymer, the dispersant polymer being a water-soluble anionic or cationic polymer which is soluble in the aqueous solution of the polyvalent ionic salt.

6. The process of claim 5, wherein the polyvalent ionic salt is a phosphate, a sulfate, or a combination comprising at least one of the foregoing salts.

7. The process of claim 1, wherein the organic, anionic or cationic, dispersion micropolymer in the salt solution exhibits a solution viscosity of greater than or equal to about 0.5 centipoise (millipascal-second).

8. The process of claim 1, wherein the organic, anionic or cationic, dispersion micropolymer in a salt solution has an ionicity of at least 5.0%.

9. The process of claim 1, wherein the siliceous material is an anionic microparticulate or nanoparticulate silica-based material.

10. The process of claim 1, wherein the siliceous material is a bentonite clay.

11. The process of claim 1, wherein the siliceous material comprises silica based particles, silica microgels, colloidal silica, silica sols, silica gels, polysilicates, aluminosilicates, polyaluminosilicates, borosilicates, polyborosilicates, zeolites, swellable clay, and combinations thereof, and wherein the siliceous material is of the material selected from the list

## 14

consisting of hectorite, smectites, montmorillonites, nonttronites, saponite, saucomite, hormites, attapulgites, laponite, sepiolites, or a combination comprising at least one of the foregoing materials.

5 12. The process of claim 1, wherein the siliceous material is introduced into the suspension before the organic micropolymer.

13. The process of claim 1, wherein the organic micropolymer is introduced into the suspension before the siliceous material.

10 14. The process of claim 1, wherein the flocculant is a cationic material selected from the group consisting of water-soluble cationic organic polymers, polyamines, poly(diallyldimethylammonium chloride), polyethyleneimine, inorganic materials such as aluminum sulfate, polyaluminum chloride, aluminum chloride trihydrate, aluminum chlorohydrate, and combinations thereof.

15 15. The process of claim 14, wherein the flocculation system additionally comprises at least one flocculant/coagulant.

20 16. The process of claim 15, wherein the flocculant/coagulant is a water-soluble polymer.

17. The process of claim 16, wherein the water-soluble polymer is formed from a water-soluble, ethylenically unsaturated monomer, or a water-soluble blend of ethylenically unsaturated monomers comprising at least one type of anionic or cationic monomers.

25 18. The process of claim 16, wherein the water-soluble polymer is a branched cationic polymer having an intrinsic viscosity greater than or equal to about 2 deciliters per gram.

19. The process of claim 1, wherein the cellulosic suspension is first flocculated by introducing the coagulating material, then is optionally subjected to mechanical shear, and then is reflocculated by introducing the siliceous material and the organic micropolymer.

30 20. The process of claim 19, wherein the cellulosic suspension is reflocculated by introducing the siliceous material before the organic micropolymer.

21. The process of claim 19, wherein the cellulosic suspension is reflocculated by introducing the organic micropolymer before the siliceous material.

35 22. The process of claim 1, wherein the cellulosic suspension comprises a filler.

23. The process of claim 22, wherein the filler is present in an amount of about 0.01 to about 50 percent by weight, based on the total dry weight of the cellulosic suspension.

40 24. The process of claim 23, wherein the filler is selected from the list consisting of precipitated calcium carbonate, ground calcium carbonate, kaolin, calcium sulphite, titanium dioxide, and combinations thereof.

25. The process of claim 1, wherein the cellulosic suspension is substantially free of filler.

26. The process of claim 1, wherein the one or more shear stages is cleaning, mixing, pumping, or a combination comprising at least one of the foregoing shear stages.

55 27. The process of claim 1, wherein the one or more shear stages comprise a centriscreen, and wherein the coagulating material is added to the cellulosic suspension before the centriscreen, and the siliceous material and organic micropolymer are added after the centriscreen.

\* \* \* \* \*